

## UNITED STATES PATENT OFFICE

2,068,088

## CASTOR OIL PRODUCT

Karl T. Steik, Upper Montclair, N. J., assignor to  
 National Oil Products Company, Harrison,  
 N. J., a corporation of New Jersey

No Drawing. Application August 27, 1934,  
 Serial No. 741,739

3 Claims.

(CL. 87—9)

My invention relates to mutual solvents for 5  
 castor oil and mineral oils and processes for pro-  
 ducing the same, and refers particularly to such  
 solvents produced from castor oil and naphthenic  
 acids.

Castor oil has valuable lubricating properties 10  
 and for many practical purposes it is advisable  
 to incorporate it in lubricating mineral oils, as  
 it increases the film strength of the lubricant,  
 thus increasing power; the oil consumption is  
 lowered and less sludge is formed by decom-  
 position when it is used.

As castor oil is insoluble in mineral oils, vari- 15  
 ous methods have been suggested to produce a  
 solution of the vegetable oil and mineral oil,  
 which processes depend generally on partially  
 decomposing the castor oil by subjecting it to  
 high pressures for prolonged periods of time,  
 with or without oxidation. These processes are  
 20 objectionable as they have a deleterious effect  
 upon the original properties of the castor oil.

It is evident, therefore, that a product which 25  
 will act as a mutual solvent for both castor oil  
 and mineral oil, and thus allow a solution of  
 the unchanged castor oil in the mineral oil,  
 would be of greatest value.

The product of my invention possesses this 30  
 valuable property, and others, as will be evi-  
 denced by a consideration of its properties as  
 herein set forth.

I have found that if castor oil be intimately 35  
 mixed with naphthenic acid and heated above  
 100° C., there results a product which acts as a  
 neutral solvent for both castor oil and mineral  
 oils and hence can be employed as a medium for  
 producing a solution of castor oil in mineral oil.

I have found that if a mixture of castor oil 40  
 and naphthenic acids in proper proportions be  
 heated above the boiling point of water, a reac-  
 tion occurs eliminating water and in which the  
 acidity of the naphthenic acids gradually dis-  
 appears and is finally neutralized.

All attempts thus far to isolate and determine 45  
 the chemical composition of the compound, or  
 compounds, thus formed have been ineffective  
 and hence I know of no way of describing it, or  
 them, except by the process of production.

It would seem however, that as castor oil is 50  
 composed mainly of triglycerides of ricinoleic  
 acid, which is an unsaturated oxy-acid, an ester  
 of this acid is formed, but I do not limit myself  
 to this particular chemical reaction, as it is stated  
 simply as an unconfirmed theory.

I have further found that the reaction between 55  
 the castor oil and the naphthenic acids takes

place slowly at the boiling point of water and, 5  
 therefore, I prefer to use a considerably higher  
 temperature, and I also prefer to use an excess  
 of castor oil in order to insure the complete  
 neutralization of the naphthenic acid.

The product of my invention has many valuable 10  
 properties, among which may be mentioned  
 the following: it is neutral, thus avoiding the  
 objectionable features of an acid lubricant; it  
 is soluble in mineral oil; it dissolves both raw 15  
 castor oil and mineral oil and thus allows a  
 neutral solution of the former in the latter; it  
 allows of the formation of non-bleeding greases;  
 it is a definite compound and hence is stable and  
 does not decompose under ordinary storage, thus 20  
 allowing the retention of the lubricating properties  
 of unchanged castor oil in the mineral oil  
 solution.

Another valuable attribute of my product is 25  
 its adaptability for textile lubricants. The diffi-  
 culty and at times impossibility of removing min-  
 eral oil droppings, or splashings, from textile  
 fibers and fabrics during their processing is a  
 source of great trouble and loss, which is greatly  
 reduced, or eliminated, in the employment of a 30  
 mineral oil solution of castor oil by means of  
 my product. If such a solution be saponified, as  
 for instance with an alkali, my compound is  
 broken down into nascent castor oil soap and  
 nascent naphthenic acid soaps and the latter 35  
 emulsifies the mineral oils, thus producing prod-  
 ucts which are readily removable from the fiber  
 or fabric.

The above-mentioned features are indicative 40  
 of the many valuable properties of my product.

As the proportions of castor oil and naphthenic 45  
 acids are dependent upon the acidity of the  
 latter, which varies greatly, it is impossible to  
 give definite quantities but these can be readily  
 determined in a practical production, because  
 the amount of castor oil present must be at least  
 sufficient to neutralize the naphthenic acids, and  
 should probably be in excess of that amount.

I give the following as one example of a proc- 50  
 ess for producing my product:

7 pounds of castor oil are added to 20 pounds  
 naphthenic acids having a neutralization value  
 of 250 and the mixture heated to 270° C. for  
 from 1 to 1½ hours. I have found that above  
 this mentioned temperature there is a tendency 55  
 for decomposition and hence excessive tempera-  
 tures are to be avoided.

In order to produce a mineral oil solution  
 of castor oil, the castor oil is dissolved in my  
 product and this solution added to mineral oil,

or my product can be added to a mixture of mineral oil and castor oil to form a solution.

As naphthenic acids are not known in a chemically pure form, but are always mixtures

5 of organic acids, saturated in nature, containing naphthenic rings and aliphatic side chains, by the words "product" or "compound" in my specification and claims, I mean the result obtained by my process.

10 As mineral oils vary from each other in their temperatures of fractional distillation, by "mineral oils" I means the distillation products of petroleum, irrespective of their individual boiling points, as for instance paraffin oil, kerosene and the heavier lubricating oils.

15 By a "neutral mutual solvent for castor oil and mineral oil" I mean a neutral product which will form a solution of the product, castor oil and mineral oil, irrespective of which compound is in fact soluble in the other.

20 I do not limit myself to the particular quan-

tities, times, temperatures, materials or steps of procedure specifically mentioned as these are given simply as a means for clearly explaining my invention.

What I claim is:

1. The product producible by heating a mixture of castor oil and naphthenic acids to a temperature above 100° C., which product is soluble in mineral oil and is a neutral mutual solvent for castor oil and mineral oil.

10 2. The product producible by heating a mixture of castor oil and naphthenic acids above the boiling temperature of water, which product is soluble in mineral oil and is a neutral mutual solvent for castor oil and mineral oil.

15 3. The product producible by heating a mixture of castor oil and naphthenic acids at a temperature of approximately 270° C., which product is soluble in mineral oil and is a neutral mutual solvent for castor oil and mineral oil.

20 KARL T. STEIK.